

Patented Jan. 4, 1927.

1,613,228

# UNITED STATES PATENT OFFICE.

HEINRICH HOZ, WALTER BERNOLLI, AND ARTHUR LINK, OF BASEL, SWITZERLAND,  
ASSIGNORS TO SOCIETY T. B. GEIGY S. A., OF BASEL, SWITZERLAND.

## PROCESS OF DYEING AND PRINTING ACETYL-CELLULOSE.

No Drawing. Application filed March 5, 1924, Serial No. 697,145, and in Germany March 31, 1923.

Hitherto known processes of dyeing acetyl-cellulose have injurious effects on the fibre. Through additions to the dyeing bath or through a convenient method of previous treatment mostly by the employment of saponifying alkalis or of organic solvents, or through too high a temperature in dyeing, the acetyl-cellulose is prejudicially altered, so that its valuable qualities are reduced or entirely destroyed.

It has now been discovered that with a large number of dyestuffs, which by themselves have only a weak affinity for acetyl-cellulose, these disadvantages can be avoided in producing the dyeing and printing of acetyl-cellulose in the presence of aryl-sulfonic acid anions. This effect can be obtained by the addition to a dye bath or printing paste of aryl-sulfonic acid compounds of any kind, in the form of free acids or salts, the dyestuffs being thus brought into a form in which they are taken up by the fibre at a relatively low temperature, which is quite harmless to the acetyl-cellulose. In this case it may be advantageous to add to the bath or paste protective colloids such as glue, gelatine, glucose, bast soap or the like, particularly with dyes which show a tendency to precipitate on the addition of organic acids.

Instead of adding aryl-sulfonic acid compounds to a dye bath or printing paste, the acetylcellulose can be previously treated with such compounds alone and afterwards, if necessary with the addition of protective colloids, dyed or printed as usual with a fresh or old bath, the essential feature being always the production of the dyeing and printing in the presence of aryl-sulfonic acid anions. The following acid compounds in the form of free acids or salts have shown themselves among others, as suitable additions: the sulfonic acids or benzol, naphthalene and anthraquinone, and their derivatives substituted by one or more oxy-, alkyl-, chloro-, or nitro-groups.

The particular working method is shown by the following examples.

### 4. For dyeing.

Example 1.—2% of methylene green and 2% of sodium diphenylamino-sulfonate are separately dissolved in water and added to the dye bath after one another at about 50° C. The acetyl-cellulose is then immersed and dyed for 3/4 of an hour at 45-50° C.,

during which the ratio of fibre to solutions is 1:60. After this, washing and further treatment is effected as usual. Carbazolsulfonic acid behaves similarly to diphenylaminosulfonic acid.

Example 2.—2% of fuchsine, having the formula



4% of gelatine and 2% of  $\beta$ -naphthalene-sulfonic acid are used in the same way as Example 1. Ratio of fibre to solution 1:60.

Example 3.—1% of pyronine G having the formula



and 1% of sodium- $\beta$ -anthroquinone-monosulfonate are used in the same way as in Example 1. Ratio of fibre to solution 1:30.

### B. For printing.

Example 4.—One part of 2,7-naphthol-sulfonic acid is dissolved by warming in 13 parts of water and mixed with 36 parts of 1:1 gum thickening. Into this paste is stirred a mixture consisting of one part of setoglaucline having the formula



dissolved in 5 parts of acetic acid of 80% strength, and 10 parts of water to which is added 34 parts of 1:1 gum thickening. The

dye paste so made is printed, steamed and washed as usual.

*Example 5.*—2 parts of sodium-1-chloro-4-naphthalene-sulfonate, are dissolved in 98 parts of water. The dry acetyl-cellulose is saturated with this padding solution and after drying printed with a dye paste which is made by dissolving 1 part of crystallized malachite green in 4 parts of acetic acid of 80% strength and 25 parts of water, and stirring in 70 parts of 1:1 gum thickening. Steaming and washing are afterwards effected as usual.

What we claim is:

15 1. A process for dyeing and printing ace-

tyl-cellulose, consisting in producing the dyeing and printing of finished acetyl-cellulose with coloring matters in the presence of aryl-sulfonic acid anions.

2. A process for dyeing and printing acetyl-cellulose, consisting in adding to the dyeing and printing mass an aryl-sulfonic acid compound and in then treating finished acetyl-cellulose with the mass thus prepared.

In witness whereof we have hereunto signed our names this 9th day of February 1924.

HEINRICH HOZ.  
WALTER BERNOULLI.  
ARTHUR LINK.